

## UNITED STATES PATENT OFFICE

2,497,890

## DRYING OILS

Peter Kass, Wilmington, Del., and Joseph Nichols,  
New York, N. Y., assignors to Interchemical  
Corporation, New York, N. Y., a corporation of  
Ohio

No Drawing. Application May 8, 1947,  
Serial No. 746,860

5 Claims. (Cl. 260—398)

1

This invention relates to the modification of drying oils by treating the oils with acetic anhydride to improve their drying qualities. The invention is particularly concerned with the treatment of mixtures of tung oil with one or more other drying oils by refluxing the mixture of oils with acetic anhydride and then removing the acetic anhydride.

Several methods for improving the drying properties of unsaturated fatty acid glyceride oils have been proposed. Among such proposed processes is one which consists in heating the oil to be modified with an oxidizing agent such as peroxide or an inorganic chromate or permanganate. A process which has been proposed for treating oilcilia oil and po-yoak oil consists in heating the oil with acetic anhydride at temperatures of 200° to 230° C. This treatment results in an increase in the drying rate of the oil.

In the copending application of Joseph Nichols, Serial Number 746,859, filed May 8, 1947, a process for treating tung oil with acetic anhydride is disclosed and claimed. It has now been discovered that when tung oil, which has been treated with acetic anhydride according to the procedure in the above application, is admixed with other drying oils commonly used in preparation of varnishes, printing inks, and the like, the beneficial effect of the acetic anhydride treatment of the tung oil is lost; the mixture of the treated tung oil with other untreated oils dried in no way different from a mixture of identical proportions of untreated tung oil and other untreated oils. We have now discovered that mixtures of tung oils and other oils will dry in the expected improved manner only if the entire mixture has been treated with acetic anhydride. This treatment with acetic anhydride may be carried out on the individual oils before mixing or it may be carried out on the mixture of oils, subsequent to mixing of the oils. The preferred procedure for carrying out our invention consists in refluxing the desired mixture of oils with 5 to 30 per cent of their weight of acetic anhydride at from about 160 to 180° C. for from about 1 to 4 hours and then removing the acetic anhydride. It is obvious that the same result is accomplished by treating the individual oils separately with acetic anhydride and then mixing them.

Our process is applicable to any mixture of tung oil with other oils, either raw or bodied, such as linseed oil, dehydrated castor oil and the like. The particular ratio of tung oil to be used with other drying oils is not critical. Such ratio will

2

be governed for the most part by the particular properties desired for the final product. High percentages of tung oil in the mixtures give a faster drying oil than a mixture containing a low percentage of tung oil.

After refluxing the mixture of tung oil and other drying oils with acetic anhydride the acetic anhydride is conveniently removed by distilling the acetic anhydride from the mixture, preferably under reduced pressure with a small stream of an inert gas such as carbon dioxide or nitrogen passing through the mixture. Although we prefer to remove the acetic anhydride under non-oxidizing conditions, we may also remove it by any other usual means, as by mere distillation or by washing the oil with water. Practically all of the acetic anhydride may be recovered.

Mixtures of tung oil with other drying oils which have been treated with acetic anhydride according to the hereinabove described process have physical properties such as viscosity, refractive index, color, etc., similar to the untreated oils; however, the treated oils dry to a tack-free film in only a fraction of the time required for the untreated oils to dry to the same degree under similar conditions. Also, the mixtures of tung oil with other drying oils, treated according to the process of our invention, tend to dry faster as the amount of tung oil in the mixture is increased. This is shown by the data contained in Table I.

Table I

| 35 | Composition of Mixture               |                                         | Drying Time          |                      |
|----|--------------------------------------|-----------------------------------------|----------------------|----------------------|
|    | Treated tung oil, per cent by weight | Treated linseed oil, per cent by weight | 25° C.               | 110° C.              |
| 40 | 30                                   | 70                                      | 2 $\frac{1}{2}$ hrs. |                      |
|    | 50                                   | 50                                      | 1 $\frac{1}{2}$ hrs. | 4 $\frac{1}{2}$ min. |
|    | 70                                   | 30                                      | 50 min.              | 1 $\frac{1}{2}$ min. |
| 45 | 90                                   | 10                                      | 35 min.              | -----                |

The drying times were determined by spreading a film of the oil on a glass microscope slide and noting the time required for the film to dry to a non-tacky state at the particular temperatures stated. Under similar conditions, mixtures of tung oil with dehydrated castor oil and soybean oil give similar results. Synthetic drying oils, for instance oils made by esterifying pentaerythritol with linseed fatty acids, also may be used in our process.

Table II shows the comparative drying times of several mixtures of treated tung oil with treated dehydrated castor oil and with untreated dehydrated castor oil.

Table II

| Composition of Mixture,<br>per cent by weight |                                       |                                     | Drying time<br>in air at<br>about 25° C. |
|-----------------------------------------------|---------------------------------------|-------------------------------------|------------------------------------------|
| treated<br>tung oil                           | untreated<br>dehydrated<br>castor oil | treated<br>dehydrated<br>castor oil |                                          |
| 90                                            | 10                                    | —                                   | 1½ hrs.                                  |
| 90                                            | —                                     | 10                                  | 35 min.                                  |
| 70                                            | 30                                    | —                                   | 2½ hrs.                                  |
| 70                                            | —                                     | 30                                  | 1½ hrs.                                  |
| 50                                            | 50                                    | —                                   | 4 hrs.                                   |
| 50                                            | —                                     | 50                                  | 2 hrs.                                   |

Table III shows the comparative drying times of several mixtures of treated tung oil with untreated soya oil and treated soya oil.

Table III

| Composition of Mixtures,<br>per cent by weight |                       |                     | Drying in<br>air at about<br>25° C. |
|------------------------------------------------|-----------------------|---------------------|-------------------------------------|
| treated<br>tung oil                            | untreated<br>soya oil | treated<br>soya oil |                                     |
| 80                                             | 20                    | —                   | 3 hrs.                              |
| 80                                             | —                     | 20                  | 40 min.                             |
| 50                                             | 50                    | —                   | 5 hrs.                              |
| 50                                             | —                     | 50                  | 2½ hrs.                             |

In addition to drying faster at room temperature the acetic anhydride treated oils also dry faster under other conditions as at a baking temperature of 110° C. or under ultraviolet light.

The improved drying oils prepared according to the process of the herein disclosed inventions are useful in the formulation of rapid drying coating compositions in the same general man-

ner as other drying oils, i. e. by mixing with solvents, coloring substances, plasticizers, other resins, and the like.

We claim:

- 5 1. A process for improving the drying qualities of mixtures of tung oil with other drying oils which comprises refluxing the mixture with acetic anhydride at 160° to 180° C. and removing the acetic anhydride.
- 10 2. A process for improving the drying qualities of mixtures of tung oil with other drying oils which comprises refluxing the mixture with acetic anhydride at 160° to 180° C. and removing the anhydride under non-oxidizing conditions.
- 15 3. A process for improving the drying qualities of mixtures of tung oil with other drying oils which comprises refluxing the mixture with acetic anhydride at 160° to 180° C. and removing the acetic anhydride under reduced pressure.
- 20 4. A process for improving the drying qualities of mixtures of tung oil with other drying oils which comprises refluxing the mixture with acetic anhydride at 160° to 180° C. and distilling the acetic anhydride under reduced pressure with the assistance of a non-oxidizing gas.
- 25 5. A process for improving the drying qualities of mixtures of tung oil with other drying oils which comprises refluxing the mixture with 5 to 30% of its weight of acetic anhydride at 160° to 180° C. and removing the acetic anhydride under reduced pressure with the assistance of a non-oxidizing gas.

PETER KASS.  
JOSEPH NICHOLS.

35

## REFERENCES CITED

The following references are of record in the file of this patent:

40

## UNITED STATES PATENTS

|           |                |              |
|-----------|----------------|--------------|
| Number    | Name           | Date         |
| 2,425,200 | Nessler et al. | Aug. 5, 1947 |